

Oct. 6, 1931.

J. H. RAMAGE

1,826,524

TREATMENT OF METALLIC FILAMENTS

Filed Nov. 10, 1927



FIG. 1.

FIG. 2.

INVENTOR  
JOHN H RAMAGE.  
BY *M T Regan*  
ATTORNEY

## UNITED STATES PATENT OFFICE

JOHN H. RAMAGE, OF BLOOMFIELD, NEW JERSEY, ASSIGNOR TO WESTINGHOUSE LAMP COMPANY, A CORPORATION OF PENNSYLVANIA

## TREATMENT OF METALLIC FILAMENTS

Application filed November 10, 1927. Serial No. 232,300.

This invention relates to the treatment of metallic filaments for incandescent lamps, electron discharge devices and similar devices and more particularly to the heat treatment 5 of tungsten filaments of the "non-sag" character, such as produced by the process set forth in Hall Patent No. 1,461,117 granted July 10, 1923, entitled Filamentary body for electric lamps and method of making the 10 same, although it may be applied to other types of refractory metal wires.

The life of a refractory metal filament is limited by alterations which take place in the filament during operation, such alteration 15 comprising rearrangement and crystalline growth within the filament and evaporation of the particles of metal from the filament. Such internal changes render the filament brittle and cause it to become deformed, that 20 is, to "sag" or "offset".

One of the objects of this invention is to impart to refractory metal wires an internal structure which resists alteration during burning and which, therefore, materially 25 adds to the operating life thereof.

Another object is to provide a heat treatment for refractory metal filaments which will increase the crystal size many times and which will very materially increase the non- 30 sag property of so-called "non-sag" wire.

A further object is to produce refractory metal filaments having an increased strength particularly when burned under vibratory conditions and which will have a long life. 35

A further object is to reduce the rate of evaporation of refractory metal filaments.

A still further object is to develop a more uniform crystal structure in a refractory metal wire.

Other objects and advantages will herein-after appear.

If a definite internal crystalline structure is imparted to a refractory metal wire before the filament is operated at or above the critical recrystallization temperature, further internal alteration is restrained and the strength and life of the material is increased.

In accordance with the present invention, I produce such internal structure by subjecting the filament after it is placed in the

envelope, to a form of heat treatment which I have discovered has the desired beneficial effect upon the filament. This heat treatment may take the place of the usual flashing or seasoning operation and consists in initially heating the wire in its strained drawn condition to temperatures which cause recrystallization. The heating is effected after mounting of the filament in the evacuated or gas filled device and is commenced at a temperature well below the recrystallization temperature. The temperature is then raised at a uniform slow rate to a point several hundred degrees above the maximum temperature at which the wire is to be heated in operation.

In metals, the grain structure of which has been deformed by mechanical working, such as drawn tungsten wire, there is a certain temperature, known as the critical or equiaxing temperature, at which the metal assumes an unstressed or natural cell-like structure, known as the equiaxed condition. Immediately above this equiaxing temperature there is a temperature zone in which the enlarging or growth of the grains composing the metal structure is extremely rapid. This recrystallization temperature varies in different types of wire depending upon the kind and purity of the materials comprising the same, the size thereof, etc., but generally speaking, recrystallization may start at about 1100° to 1400° C. for tungsten filaments of the non-sag type.

I have found that if the initial heating of the drawn wire is commenced at a temperature below this recrystallization temperature and slowly and uniformly raised therethrough that a crystal structure is developed in which the crystals are of very large size and which retain their interlocking or non-sag character. The slow heat treatment gives the crystals sufficient time to grow enormously in the zone of rapid grain growth and the uniform increase in temperature produces a temperature gradient between adjacent grains extending from the point or points of highest temperature to the point or points of lower temperature. Due to the loss of heat by conduction at the filament supports or leads,

there is always a point on the filament between such supports or leads where the filament attains the highest temperature. As the temperature of the filament is slowly raised from a temperature below the recrystallization temperature these points of highest temperature are the first to reach the condition favorable for grain growth and due to the temperature gradient existing between the grains at these points and the adjacent grains, there is an absorption of the cooler grains by the higher temperatured ones whereby the grain of higher temperature increases in size. This increase in size further augments the grain absorbing power of the crystal of higher temperature so that its growth is accelerated. As the temperature further increases the outlying grains gradually reach the recrystallization temperature and the growth continues outwardly in each direction from the point or points of maximum temperature until growth of the crystal is arrested by contact with another crystal of such size that it cannot be absorbed.

The rate of increase of temperature depends upon the size of the wire being treated but in general a shorter time than 3 minutes does not give the satisfactory results even with the smallest sizes of filaments when mounted in lamps as coiled filaments and for sizes above 3 mil diameter the time required to raise the temperature from below the recrystallization temperature to a point well above the normal operating temperature should be increased at the rate of about 1 minute per mil of increased diameter.

For example, in the case of a 50 watt, 115 volt tungsten filament, which normally burns at a current of .435 amperes, the initial lighting current was about .087 amperes and by means of an adjustable resistance the current was raised at a uniform rate over a period of 3 minutes to about .582 amperes. Lamps having their filament treated according to this schedule had a life under vibratory operation conditions of twice that of lamps flashed according to the schedule heretofore employed. The schedule heretofore employed consisted of a short flash at 100 and 130% of normal operating voltage.

As an example of the treating schedule employed on large wire, a good interlocking crystal of large size was obtained in a 25 mil wire operating at a normal current of 24 amperes, by raising the current from 2 amperes to 26 amperes in about 20 minutes, and in the case of a 40 mil wire, normally operating at 52 amperes, by raising the current from 10 amperes to 58 amperes in 30 minutes, although good results were obtained in this last instance with a 20 minute schedule.

The effects of this initial slow uniform increase in temperature appear to be to develop a larger grain structure and a more uniform good crystal structure having interlocking

grain boundaries which are more resistant to offsetting and furthermore, to the development of this structure in the parts of the filament which are ordinarily chilled, i. e., at the lead connections and across the filament supports. The high finishing temperature promotes the last feature and is not necessary when no cooled parts are present in the span to be treated. However, to prevent further crystal alteration during the operation of the filament, it should be heated to a temperature above the maximum temperature to which it will be subsequently subjected during operation.

In order to insure that the heat treatment will commence well below the critical recrystallization temperature and continue well above the maximum temperature which the filament will attain during use, I prefer to start the treatment at a temperature of about 800° C. and to continue the treatment up to a temperature several hundred degrees above the normal operating temperature of the filament. The maximum treating temperature may vary between 2200° C. and 2800° C. depending upon the use to which the filament is to be subjected.

The treating current must be applied continuously and without interruption until a temperature is obtained sufficiently high to carry the crystallization around the cold portions of the filament supports. An intermittent schedule does not produce the same results in crystal formation, since when the filament is heated by intermittent steps, the crystallization takes place at the first step at which the temperature is within the critical grain growth range and immediately ceases again when the current is cut off in switching to the next step and the filament momentarily cools. The subsequent steps have little effect as the grain growth and temperature gradients are interrupted at each step change.

In order that the effect of the heat treatment herein described can be more fully understood, reference will be had to the accompanying drawings in which:

Fig. 1 is a longitudinal sectional view of a recrystallized non-sag filament flashed by the method heretofore employed and showing the usual crystal structure thereof; and,

Fig. 2 is a longitudinal sectional view of a recrystallized non-sag wire treated in accordance with my invention and showing the exaggerated crystal structure obtained thereby.

Referring to Fig. 1, it will be noted that the crystal structure comprises a large number of very fine grains 10. The size of the grains can be better appreciated when it is understood that the figures represent photomicrographs of a 25 mil wire taken at a magnification of about 75 diameters. The crystals shown at 11 in Figure 2 illustrate the

growth that has taken place during the slow continuous increase in temperature which is described above. It should be noted that many of the crystals 11 have an extent of 5 substantially half the diameter of the wire or about 10 mil in diameter and a length of many times the diameter. In many instances, I have obtained single crystals extending over the entire diameter of the wire, 10 and in larger size wires of as high as 40 mil or greater.

Referring to Figure 1, the dark portions 12 shown extending along each side of the wire are not a representation of single crystals but illustrate the receding curved portion or rounded edge of the wire, as it appears in the original photo-micrograph.

It is understood that many changes may be made in the treatment and that it may be 20 applied to various types of wire and I do not desire to be limited to the exact details described but contemplate such modifications as come within the scope of the invention as defined in the appended claims.

25 What is claimed is:

1. The method of treating tungsten wire to promote the development of large crystals comprising initially subjecting the drawn wire to a temperature about 800° C. and increasing the temperature at a slow rate up to 30 a point above the normal operating temperature.
2. The method of treating non-sag tungsten wire to increase the crystal size and augment the non-sag property of the wire comprising elevating the temperature of the wire from below 1100° C. to above 2200° C. at a substantially uniform rate, over a period of approximately one minute per mil diameter 40 of the wire.

In testimony whereof, I have hereunto subscribed my name this 9th day of November, 1927.

JOHN H. RAMAGE.